

# United States Patent

[19]

[11] 3,883,356

Syrovatka et al.

[45] May 13, 1975

[54] RINSE-WAX FORMULATION

[75] Inventors: Rudolf Syrovatka; Kurt Hofer, both of Vienna, Austria

[73] Assignee: Lever Brothers Company, New York, N.Y.

[22] Filed: Apr. 9, 1973

[21] Appl. No.: 349,165

[30] Foreign Application Priority Data

Apr. 11, 1972 United Kingdom..... 16591/72

[52] U.S. Cl. .... 106/8; 106/11; 106/267

[51] Int. Cl. .... C08h 9/00; C09d 1/14

[58] Field of Search ..... 106/8, 247, 285, 243; 252/312; 117/134

[56] References Cited

UNITED STATES PATENTS

2,765,255 10/1956 Swarbrick ..... 252/312

|           |         |               |         |
|-----------|---------|---------------|---------|
| 2,956,971 | 10/1960 | Lam.....      | 106/243 |
| 3,222,201 | 12/1965 | Boyle.....    | 252/312 |
| 3,497,365 | 2/1970  | Atherton..... | 106/8   |

## OTHER PUBLICATIONS

The Chemical Dictionary, p. 107, 1961.

Primary Examiner—Theodore Morris  
Attorney, Agent, or Firm—James J. Farrell, Esq.;  
Melvin H. Kurtz, Esq.; Arnold Grant, Esq.

[57]

## ABSTRACT

Rinse-wax formulation suitable for incorporation into rinse waters during the laundering of cars and automobiles, comprising a cationic surfactant, a mineral oil, a non-alkalimetal soap and water, wherein the mineral oil constitutes a mixture of paraffinic and aromatic/naphthenic material.

5 Claims, No Drawings

## RINSE-WAX FORMULATION

## BACKGROUND OF THE INVENTION

## 1. Field of the Invention

This invention relates to a rinsing formulation for treating cleaned surfaces. More particularly it relates to a so-called rinse-wax formulation for rinsing previously cleaned cars and automobiles.

Automobiles and the like are generally washed and cleaned with alkaline "built" detergents or anionic detergents. After application of the detergent the automobile finish is rinsed and dried in the conventional manner, i.e., with a cloth or by means of an air blast. A rinsing formulation is generally added to the last rinsing water to facilitate the rinsing and drying of the cleaned surfaces and provide a deposit of a water-repellent film on the treated surface.

## 2. Description of the Prior Art

A rinsing formulation comprising an oil-in-water emulsion containing a cationic surfactant, a mineral oil and water is known from U.S. Pat. No. 3,222,213. In U.S. Pat. No. 3,497,365 the addition of wax and/or silicones is suggested to effect an additional protective film.

A serious drawback of using these additives in rinse formulations is that these additives tend to stick and form a very annoying layer onto the windshield and windows of cars and automobiles, obscuring the driver's view.

## SUMMARY OF THE INVENTION

It is an object of the present invention to provide a rinse-wax formulation with an improved hydrophobing effect, without having the above drawback.

It is another object of this invention to provide a rinse-wax formulation, which provides a stable hydrophobic film-finish onto cars and automobiles, rinsed therewith.

Still another object of this invention is to provide a clear liquid rinse-wax formulation which has satisfactory cold-stability.

Accordingly, the present invention provides an improved rinse-wax formulation, which comprises essentially a cationic surfactant, a metal soap, a mineral oil, and water.

## DESCRIPTION OF THE INVENTION

It has been found that an improved rinse-wax formulation suitable for incorporation into rinse-waters during the laundering of cars and automobiles, comprising a cationic surfactant, a mineral oil and water, can be prepared by the addition of low levels of a non-alkalimetal soap of long chain fatty acids in combination with a mixed paraffinic and aromatic/naphthenic mineral oil.

Accordingly the rinse-wax formulation of the present invention comprises a cationic surfactant, a mineral oil constituting a mixture of paraffinic and aromatic/naphthenic material, a non-alkalimetal soap of long chain fatty acids, and water.

The cationic surfactants which can be used in the formulation of the invention are known and generally will be nitrogen-containing compounds which are reaction products of long-chain fatty acids containing from 8 to 22 carbon atoms with alkylene polyamines, alkylol amines or ammonia; the condensation products of a primary fatty amine containing from 8 to 22 carbon

atoms with alkylene oxide, such as ethylene oxide or other active epoxides, such as propylene oxide and the like; and the quaternary ammonium salts of fatty amines having at least one alkyl substituent containing from 8 to 22 carbon atoms such as fatty amine acetates, fatty amine chlorides, fatty amine bromides and the like.

Typical illustrative nitrogen-containing compounds which are the reaction products of long-chain fatty acids with alkylene polyamines are 1-(2-amino ethyl)-2-heptadecenyl-2-imidazoline; 1-(2-amino ethyl)-2-heptadecadienyl-2-imidazoline, and the like.

Typical reaction products of long-chain fatty acids with alkylol amines are 1-(2-hydroxyethyl)-2-heptadecenyl-2-imidazoline; 1-(2-hydroxyethyl)-2-heptadecadienyl-2-imidazoline, and the like.

Typical reaction products of long-chain fatty acids with ammonia are octadecylamide, hexadecylamide, docosylamide, octylamide, and the like.

Typical condensation products of a primary fatty amine with an alkylene oxide or the like are the N,N-di-(mono- and polyalkylene-oxyalkylol)-octadecylamines, the N,N-di-(mono- and polyalkylene-oxyalkylol)-heptadecylamines, the N,N-di(mono- and polyalkylene-oxyalkylol)-hexadecylamines, the N,N-di-(mono- and polyalkylene-oxyalkylol)-tetradecylamines, the N,N-di(mono- and polyalkylene-oxyalkylol)-dodecylamines, and the like.

Typical quaternary ammonium salts are the coconut oil quaternary amine acetates, octadecyltrimethylammonium chloride, octadecylbenzylidemethylammonium chloride, hexadecyldimethylammonium bromide, dodecyl trimethylammonium chloride, and the like.

The preferred cationic surfactants for the instant formulations are the quaternary ammonium salts of fatty amines having at least one alkyl substituent containing from 8 to 22 carbon atoms. Particularly preferred are the coconut fatty amine acetates.

By the term "metal soap" as used herein is meant the non-alkali metal salts of long-chain fatty acids having about 12-22 carbon atoms. It has been established that by the presence of small amounts of metal soap the properties of rinse-wax formulations are greatly improved. Suitable metal soaps for the formulation of the invention are the fatty acid salts of metals of Group IIA, IIB and IIIA of the periodic system, such as the Mg-, Ca-, Sr-, Ba-, Zn-, Cd- and Al-soaps, of which the stearates are particularly preferred. Metal stearates are for example derived from hardened tallow fatty acids, and technical or pure grade stearic acid, comprising a mixture of predominantly C<sub>16</sub>-C<sub>18</sub> saturated fatty acids.

The mineral oils suitable for the formulation of the invention are the mixed paraffinic and aromatic/naphthenic mineral oils. It is essential that the mineral oil used in the invention contains a certain proportion of aromatic/naphthenic constituents, to get the benefit of the effect from the metal soap constituent in the formulation. Surprisingly it has been observed that either pure paraffine mineral oil or pure aromatic/naphthenic mineral oil is not suitable for the purpose of the invention, since compositions with or without metal soaps comprising these oils would have substantially equal performance. The combined effect of mixed oils and metal soap is quite surprising. Preferred mineral oils are those having an aromatic/naphthenic content within the range of from about 5-70% by weight, more preferably from 15-50%. In practice the mineral oil

employed will have a boiling point of at least 100°C, since lower boiling oils would be too volatile.

Preferably the formulation contains a solubilizing nonionic substance. Whereas this latter is not essential to the technical performance of the product, it does promote the solubilization of the mineral oil and other essential ingredients in the aqueous medium, thus making the formulation more manageable and more suitable for use.

The rinse-wax formulation according to the invention therefore comprises an effective amount of cationic surfactant, a non-alkali metal soap derived from long chain fatty acids, a mineral oil constituting a mixture of paraffinic and aromatic/naphthenic material and water. In one preferred embodiment of the invention a substantially clear liquid rinse-wax formulation is provided, containing a solubilizing nonionic substance.

The term "solubilizing nonionic substance" is used herein to indicate a non-detergent organic nonionic material having solubilizing properties. Specifically contemplated within this definition are the lower ethoxylated nonionics containing 2-4 ethylene oxide groups per molecule; the glycols and their derivatives, such as ethylene glycol, diethylene glycol, butyldiglycol, and the like; the low-molecular weight monohydroxy alcohols, such as butanol and isobutanol, and mixtures thereof.

In a rinse-wax formulation of the invention, the cationic surfactant may be present in amounts in the range of 1-20% by weight, the preferred range being from 2-10% by weight. The metal soap is present in the formulation usually in an amount in the range of 0.01-2.0% by weight and preferably in an amount from about 0.05-0.75% by weight. The mineral oil as hereinbefore defined is present usually in an amount of at least 10% by weight up to about 30% by weight of the formulation. Preferably the formulation of the invention contains aromatic/naphthenic oil material within the range of from about 0.5-10% by weight, preferably

from 0.5-6.0% by weight, based on the total composition prior to dilution.

The amount of solubilizing nonionics preferably employed in the formulation is about 5-15% by weight.

Other ingredients may also be added in the formulation, if desirable, such as for example low-foaming nonionic surfactants, perfume, colouring substances, etc.

The rinse-wax formulation according to the invention is applied to the cars in the conventional manner by diluting it with water in a ratio of the order of about 1:1,000 and spraying it onto the cars after they have been washed and rinsed, or while they are being rinsed.

Surprisingly rinse-wax compositions formulated as herein described according to the invention show remarkably better properties and performance on use as compared with the conventional compositions, particularly with respect to water-break- and hydrophobing effect, and film stability.

Whereas some conventional rinse-wax formulations are relatively sensitive to the hardness of the water used for rinsing, the performance of the formulation of the invention is substantially unaffected when used in either soft or hard water.

A noticeable improvement in cold-stability has also been observed.

A further improvement is that rinse-wax formulations of the invention maintain their effectiveness irrespective of the type of detergents used in the cleaning and washing stage of the vehicle, i.e., not susceptible to anionic detergents.

Typical rinse-wax formulations and their properties are illustrated in the following Examples; which are not to be considered as limitative in any respect.

### EXAMPLES I - III

Formulations I, II and III within the invention compared with Formulations A, B and C as regards hydrophobing effect and stability of the hydrophobic film.

The results are tabulated below:

| Ingredients:                                                                 | I    | II   | III  | Formulation in % by weight |       |       |
|------------------------------------------------------------------------------|------|------|------|----------------------------|-------|-------|
|                                                                              |      |      |      | A                          | B     | C     |
| Mineral oil with an aromatic/naphthenic content of 25%                       | 12.5 | —    | —    | 12.5                       | —     | —     |
| Mineral oil with an aromatic/naphthenic content of 55%                       | —    | 12.5 | 12.5 | —                          | —     | —     |
| Mineral oil free from aromatic/naphthenic compounds                          | —    | —    | —    | —                          | 12.5  | 12.5  |
| Coconut fatty amine acetate                                                  | 5.0  | 5.0  | 10.0 | 5.0                        | 10.0  | 10.0  |
| Mixture of Al- and Mg-Stearate *                                             | 0.1  | 0.5  | —    | —                          | —     | 0.5   |
| Mixture of Al- and Zn-Stearate *                                             | —    | —    | 0.5  | —                          | 0.5   | —     |
| Fatty alcohol polyethylene glycol ether containing 5 moles of ethylene oxide | 9.0  | 12.0 | 12.0 | 9.0                        | 12.0  | 12.0  |
| Isopropanol                                                                  | —    | —    | —    | 7.0                        | —     | —     |
| Diethylene glycol                                                            | 2.5  | —    | —    | —                          | —     | —     |
| Isobutanol                                                                   | 4.5  | —    | —    | —                          | —     | —     |
| Butyldiglycol                                                                | —    | 4.5  | 4.5  | —                          | 4.5   | 4.5   |
| Ethylene glycol                                                              | —    | 5.0  | 5.0  | —                          | 5.0   | 5.0   |
| Water                                                                        | 66.4 | 60.5 | 55.5 | 66.5                       | 55.5  | 55.5  |
| Properties                                                                   |      |      |      |                            |       |       |
| Hydrophobing effect <sup>1)</sup> (water break)                              | 15   | 10   | 15   | >50                        | >50   | >50   |
| Stability of the <sup>2)</sup> hydrophobic film                              | 360  | 400  | 380  | 10-15                      | 20-30 | 20-30 |

<sup>1)</sup>Expressed as number of drops of a rinse wax solution (conc. 2 g/l) from a burette necessary for water break on a lacquered surface being wetted before with a solution of 0.2 g/l sodium-alkylbenzene sulphonate.

<sup>2)</sup>Expressed in minutes necessary for re-wetting by spraying water onto a hydrophobized surface.

The above Table shows that formulations I, II and III according to the invention were clearly better than formulations A, B and C which are outside the scope of the present invention.

The above formulations I - III can be diluted with water in a ratio of about 1-2 parts of the formulation to about 1,000 parts of water and sprayed on cleaned cars prior to drying.

Similar results were obtained when the coconut fatty amine acetate in the formulation was replaced by:

1. tallow fatty amine-ethoxylates with 5 moles of ethylene oxide;

2. octadecylamide.

What is claimed is:

1. A rinse-wax formulation suitable for incorporation into rinse waters during the laundering of cars or automobiles, comprising an aqueous medium having therein solubilized a cationic surfactant selected from the group consisting of reaction products of long-chain fatty acids containing from 8-22 carbon atoms with alkylene polyamines, alkylolamines or ammonia, the condensation products of primary fatty amines containing from 8-22 carbon atoms with an alkylene oxide, the quaternary ammonium salts of fatty amines having at least one alkyl substituent containing from 8-22 carbon atoms; and mixtures thereof; a mineral oil having an aromatic material content of from about 15-70% by weight; and a non-alkalimetal salt of long chain fatty acids having from about 12-22 carbon atoms in the chain, selected from the group consisting of magnesium, calcium, strontium, barium, zinc, cadmium, aluminum salts and mixtures thereof; said formulation comprising essentially about 1-20% by weight of said cationic surfactant, about 10-30% by weight of said mineral oil, about 0.01-2.0% by weight of said non-alkalimetal soap, and the balance water.

2. A substantially clear liquid rinse-wax formulation suitable for incorporation into rinse waters during the laundering of cars or automobiles, comprising an aqueous medium having therein solubilized a cationic surfactant selected from the group consisting of reaction products of long-chain fatty acids containing from 8-22 carbon atoms with alkylene polyamines, alkylolamines or ammonia, the condensation products of primary fatty amines containing from 8-22 carbon atoms with

5 an alkylene oxide, the quaternary ammonium salts of fatty amines having at least one alkyl substituent containing from 8-22 carbon atoms; and mixtures thereof; said formulation comprising essentially about 1-20% by weight of said cationic surfactant, about 10-30% by

10 weight of said mineral oil, about 0.01-2.0% by weight of said non-alkali metal soap, about 5-15% by weight of a solubilizing nonionic substance, selected from the group consisting of non-detergent lower ethoxylated nonionic compounds having from 2-4 ethylene oxide

15 groups per molecule, glycols and their derivatives selected from the group consisting of ethylene glycol, diethylene glycol and butyldiglycol, butanols and mixtures thereof, and the balance water.

20 3. A rinse-wax formulation according to claim 1, which contains about 0.5-10% by weight of aromatic/naphthenic oil based on the total composition.

25 4. A rinse-wax formulation according to claim 1, in which the non-alkali metal soap is present in an amount 30 from about 0.05-0.75% by weight of the total formulation.

35 5. A rinse-wax formulation according to claim 1, in which the cationic surfactant is a coconut fatty amine acetate.

\* \* \* \* \*